

Aug. 22, 1933.

W. O. SNELLING ET AL

1,923,761

MANUFACTURE OF DETONATING FUSE

Filed July 28, 1932

FIG. 1



FIG. 2



FIG. 3



WALTER O. SNELLING  
CLARENCE B. KOCH  
INVENTORS

BY

Walter O. Snelling,  
ATTORNEY

## UNITED STATES PATENT OFFICE

1,923,761

## MANUFACTURE OF DETONATING FUSE

Walter O. Snelling and Clarence B. Koch, Allentown, Pa., assignors to Trojan Powder Company, a Corporation of New York

Application July 28, 1932. Serial No. 625,340

4 Claims. (Cl. 102—8)

Our invention relates to improvements in the manufacture of detonating fuse, and more particularly relates to the preparation of detonating fuse of improved ability to withstand long continued storage without loss of sensitiveness. The principal object of our invention is to provide means for the manufacture of detonating fuse or "cordeau" of initial high sensitiveness, and which maintains this initial high sensitiveness 10 without substantial diminution with time.

Detonating fuse or cordeau consists of an outer tube or sheath of tin, lead, or any other suitable metal or alloy, and an inner core or member of trinitrotoluene, trinitrobenzene, tetryl, pentaerythrite tetranitrate or any other suitable detonating agent or mixture of detonating agents. Detonating fuse is made by filling the outer sheath or tube with a molten charge of the fused detonating agent, permitting this fused charge to 20 solidify, and then increasing the length and decreasing the diameter of the composite tube by a series of rolling or drawing operations as described in U. S. Patent 869,219 of October 22, 1907 to Lheure or U. S. Patent 882,154 of March 25, 1908 to Lheure, or by increasing the length and decreasing the diameter of the composite tube by a swaging operation, as described in U. S. Patent 1,741,380 of December 31, 1929 to Snelling and Koch.

It has been found that detonating fuse or cordeau made by either of the methods known up to this time has satisfactory sensitiveness at the time of its manufacture, when made with trinitrotoluene or other detonating agent of high purity, but with age this initial high sensitiveness gradually decreases, so that detonating fuse or cordeau several years after its manufacture often shows insufficient sensitiveness to enable 35 the detonating wave to propagate completely through the material, and failure to detonate past junctions and connections of trunk lines with subsidiary lines of cordeau are of frequent occurrence.

Discovery of the fact that detonating fuse or cordeau which has been stored for some time shows reduced sensitiveness is not new, but on the contrary has been recognized for many years as being one of the outstanding disadvantages 50 of an otherwise excellent means of simultaneously transmitting detonation to a number of separating charges of high explosives. It has been discovered that by the use of refined trinitrotoluene of exceptional purity the tendency toward reduction of sensitiveness with time can

be avoided to a considerable extent, and it has also been discovered that the admixture of a more sensitive detonating agent than trinitrotoluene with the trinitrotoluene used as the principal detonating charge in cordeau also results in 60 improved keeping properties or ability to withstand storage without excessive loss of sensitiveness, as has been pointed out in U. S. Patent 1,241,705 of June 1, 1920 to Cope.

We have discovered means by which detonating 65 fuse or cordeau of improved sensitiveness can be produced in an extremely simple and inexpensive way, and the cordeau produced by our new method possesses exceptional ability to withstand long continued storage without reduction in sensitiveness with time.

In order to explain the novel features involved in our present invention we will now point out certain relationships which exist in cordeau made by the methods at present known, in order to 75 distinguish these relationships from the corresponding relationships existing in cordeau made by our present invention. In the manufacture of cordeau by the methods known up to this time, a metal tube is filled with a molten detonating 80 agent, and is then increased in length and decreased in diameter by a series of rolling, drawing or swaging operations, until cordeau of the desired final diameter is secured. It is imperative that the tube should be completely filled with the 85 molten detonating agent, since any large air bubble or interruption in the explosive core will of course lengthen materially in the rolling, drawing or swaging operations, and will prevent the satisfactory functioning of the finished fuse, through 90 inability of the relatively weak detonating force of the thin core of trinitrotoluene to jump any gap or open space in the column of explosive material.

Accordingly, in all cordeau which has been 95 made up to the date of this invention, there has been a direct and necessary relationship between the initial diameter of the cordeau, the final diameter of the cordeau, and the density of the contained charge of trinitrotoluene or other detonating agent used. The initial tube, before being drawn down or swaged down to its final diameter, is filled with the molten detonating agent which solidifies within the tube to form the solid detonating agent at its normal density when 105 solidified from fused condition. The operations of drawing or swaging the filled tube, to decrease its diameter and increase its length, breaks up the fused detonating charge and reduces it to a 110 pulverulent condition, with the production of a

highly compressed pulverulent mass within the lead tube, the exact density of this pulverulent mass being determined by the volume and pressure relationships existing during the drawing and swaging operations. For example, when lead tube 16 mm. inside diameter and 19.5 mm. outside diameter is filled with molten trinitrotoluene of high purity, and this trinitrotoluene is then allowed to cool and solidify, the density of the 5 fused trinitrotoluene within the tube is initially about 1.60. Upon drawing this initial tube down to a final outer diameter of 6 mm., corresponding to an inner diameter of 4.25 mm. and a wall thickness of 0.875 mm., the pulverulent charge of 10 trinitrotoluene within the finished cordeau has a density of approximately 1.30, and it is interesting to note that up to the time of the present invention no method was known of modifying this 15 density, since the density of the main charge of 20 pulverulent trinitrotoluene was a definite and necessary factor of the drawing or swaging operation used in manufacturing the detonating fuse or cordeau. According to the initial diameter of 25 the lead tube and the final diameter of the finished cordeau, the charging density of the pulverulent trinitrotoluene in ordinary commercial 30 cordeau having an outer diameter of 6 mm. shows a normal variation in cordeau made by the drawing operation of from 1.20 to 1.30, and shows a 35 normal variation in cordeau made by the swaging operation of from 1.30 to 1.40, the density of the pulverulent charge of trinitrotoluene in cordeau made by the swaging operation being somewhat greater than the density of the charge in cordeau 40 made by the drawing operation, because of the greater pressure applied to the trinitrotoluene core in the swaging operation, as compared with the corresponding pressure produced in the drawing operation.

45 It has long been known that the sensitiveness to detonation of many explosives is materially influenced by the density of the material, and some explosives are well known to become highly insensitive when subjected to high pressure. Up to 50 the time of the present invention, however, the density of the pulverulent charge of trinitrotoluene in cordeau has never been considered to have significance, in view of the fact that whether 55 cordeau is made by the drawing process or by the swaging process it shows satisfactory initial sensitiveness, and shows no indications whatever of being excessively compressed or of being charged to so high a density as to interfere with the normal progress of the detonating wave.

60 We have discovered, however, that although the initial sensitiveness of pulverulent trinitrotoluene is not measurably influenced by the density of the pulverulent material, this is not true 65 of the sensitiveness after storage for any considerable length of time. Apparently, the closeness of contact of the pulverulent particles determines the degree to which recrystallization of the material occurs, the finely divided pulverulent 70 particles ultimately agglomerating or consolidating, and partially recrystallizing or reforming into particles of larger crystal size, with very serious reduction in sensitiveness, and the reduction in sensitiveness being materially greater 75 in the case of trinitrotoluene of a melting point under 80° C. than it is with trinitrotoluene having a melting point higher than this figure, desensitization with time being determined by the percentage of impurity present in the detonating 80 charge, and being materially greater in the case

of slightly impure trinitrotoluene than it is in the case of trinitrotoluene of high purity.

Our studies of the effect of time on the sensitiveness of cordeau indicated the desirability of modifying the density of the inner core of cordeau independently of the reduction which is determined by the operations of drawing down or swaging down the original tube to the desired final dimensions, but all efforts to introduce light porous filling materials, air bubbles, foam or the like as a means of reducing the density of the core proved unsuccessful, and all known methods of drawing, rolling and swaging the outer tube were found to produce definite correlated densities in the inner core of explosive material. 85 90

We have now discovered a method by which we can modify the density of the inner core of explosive material independently of the degree of reduction or "drawing down" of the outer tube or casing, and our method is capable of controllably modifying the density of the inner core of explosive material over a satisfactorily wide range to enable us to obtain cordeau of longer effective life without decreasing sensitiveness than can be obtained by any of the methods previously known. 95 100

In the simplest form of our invention we first distort a tube by a preliminary rolling or pressing operation so that this tube is no longer circular in cross-section. Although we prefer to distort the 105 tube so that after distortion it is elliptical in cross-section, it will of course be evident that a circle forms the figure which has maximum area for any given periphery, and that accordingly any uniform deviation from a circle will produce 110 a figure in which the relationship between the cross-sectional area and periphery will be reduced, as compared to the relationship which exists in a circular tube. We prefer to distort our metal tubing to form an ellipse in which the 115 major diameter is between 1½ and 3½ times the minor diameter, and we next fill this tube with molten trinitrotoluene while it is in such uniformly distorted condition along its entire length. The molten TNT is permitted to harden 120 in the usual way while the tube is in its distorted condition, and the distorted tube containing its solidified core of trinitrotoluene or other explosive agent is then subjected to a rolling or pressing operation to restore it to circular form. Upon 125 being so restored to circular form the outer tube or casing possesses substantially the circumference of the original tube, but the amount of contained trinitrotoluene corresponds only to the reduced cross-sectional area of the ellipse which 130 existed at the time the tube was filled with the molten detonating material, and accordingly the density of the contained trinitrotoluene is correspondingly reduced. Upon now subjecting the 135 tube with its contained core of explosive material to rolling, drawing, or swaging operations to reduce its diameter to the diameter desired in the final cordeau there occurs a tendency to constantly approach the usual ratio of the diameter 140 to the density met with in ordinary cordeau, although this ratio is never quite reached, owing to the initial advantage obtained as a result of the reduced filling density obtained as a result of the novel filling method as herein described. The larger the initial diameter of the lead tube, 145 and the less the distance between the foci of the ellipse, the higher will be the final density of the explosive core in the finished cordeau, and accordingly by suitable control of the diameter of the original lead tube, and suitable distortion of 150

this tubing in the formation of the initial ellipse which is filled with molten trinitrotoluene, we can control the density of the finished explosive core in our cordeau within a satisfactory range to give us cordeau which resists storage for many months at temperatures corresponding to the maximum summer temperatures met with in storage magazines, without any perceptible reduction in sensitiveness occurring.

10 In the drawing forming part of this application Figure 1 is a cross-sectional view of a lead tube filled with trinitrotoluene in accordance with the usual procedure followed in the manufacture of cordeau. Figure 2 is a cross-section of a lead tube filled with trinitrotoluene in accordance with the procedure which we have discovered. Figure 15 3 is a cross-section of the tube shown in Figure 2, after this tubing has been restored to circular outline. In all of the figures, A is the outer tubing of lead, tin or other metal. In all of the figures B is the core of trinitrotoluene or other explosive mixture.

The material of which the outer tube or casing is made does not form any part of our present 25 invention, and although we prefer to employ lead as the material from which the outer tube or casing is made, it will be evident that other metals, and particularly other ductile metals such as tin and copper, or alloys of lead and tin, lead and 30 antimony, or lead, tin, and antimony may be used with equal success. We may also employ, in cases where such procedure may be desirable, a composite tube formed with an outer layer of a metal such as lead and an inner member of 35 tin or other metal, such composite tube having advantages in cases where the explosive material has any tendency to react with the metal forming the body of the outer tube or casing. As our explosive core we prefer to employ trinitrotoluene, 40 but we may employ any other suitable detonating agent such as picric acid, tetryl, or the like.

We are of course aware that in the manufacture 45 of cordeau prior to our invention it is quite possible, and indeed is most likely, that some portions 50 of the lead tube may have accidentally become distorted in form through injury in handling, and that notwithstanding the careful inspection which is usually given to the tubing before being filled with trinitrotoluene, it is quite likely that at times 55 tubing which has been locally thus injured and distorted at one or more points along its length may have been filled with trinitrotoluene and may have been manufactured in finished cordeau. In view of the possibility just stated, we 60 wish to expressly disclaim as any part of our invention the manufacture of cordeau from tubing which has been subjected to such accidental injury, and we wish to state that our invention is to be considered as limited to the process which 65 comprises the uniform distortion of tubing along substantially its entire length before being filled, and the uniform filling of such distorted tubing to form a non-circular tube having substantially the same cross-section at all points along its length, and possessing at all points along its 70 length a cross-sectional area greater than the area of a circle corresponding to the normal diameter of the lead tubing used.

During our investigation of the manufacture 75 of cordeau by the method herein described we have discovered an important advantage of our present method of manufacture which we did not know at the time that we began our work, but which became evident in the course of our investigation of cordeau made by our present process.

We have discovered that the tendency of the outer tubing to break or fracture during manufacture or as a result of flexure during or after manufacture is greatly reduced in cordeau made by our present process as compared with cordeau made by the processes in use up to the time of our present invention. Although at first we could find no reason to explain the greater strength of the outer casing of cordeau when made by our present invention, as compared with cordeau as made by the methods earlier known, we have now found that during the solidification of trinitrotoluene or other crystalline detonating agent within the tube used in the manufacture of cordeau the crystals which form are somewhat harder than the boundaries between these crystals, and that when the filled tube is subjected to operations to decrease its diameter and increase its length the effect of the pressure applied to the tube is to cause the crystalline mass to form indentations on the inner wall of the tubing proportional to the hardness of the individual crystal particles at such points, so that tubing after initial treatment when subjected to heat to remove the inner core shows a noticeably roughened surface. Upon being subjected to further treatment to increase its length and decrease its diameter, these initial roughnesses form the source of differences of thicknesses in the wall of the finished cordeau, and owing to the great increase in length 100 and decrease in diameter which occurs in the drawing operation, even a furrow or indentation of very minor depth becomes a source of considerable weakness in the tube after the wall thickness has been reduced to its final limit. We 105 have discovered that when a distorted tube prepared in accordance with our present invention is subjected to a preliminary operation to break up the contained solid core by applying pressure to the distorted tube the contained solid core of 110 trinitrotoluene breaks up into pulverulent material without similarly indenting the inner lead wall, no doubt because of the fact that the nature of the distortion of the tube permits of relief to the shearing forces applied to the crystals due 115 to the distortion of the tube producing simultaneously modified and increased cross-sectional area available for expansion of the material. As a result of this condition, which we discovered accidentally during the course of our work, we 120 are able to produce by our present process of manufacture not only cordeau of materially improved sensitiveness, but also cordeau which possesses a notably stronger outer metal wall than 125 is produced by other methods of manufacture, and we have found that the tendency of the lead wall of our cordeau to pierce or break or fracture during manufacture or subsequent to manufacture when subjected to bending or other action 130 is notably reduced as compared with cordeau made by the process of manufacture known and practiced up to the time of our present invention. 135 Although we prefer to use ordinary lead pipe or tubing as our raw material, and to distort this lead tubing to elliptical or non-circular cross-section by means of rolls, it will of course be evident that the step of distorting circular tubing to non-circular cross-section does not form an essential feature of our invention in view of the fact that it is quite easy by methods well known 140 in the art to initially produce lead tubing by an extruding operation directly in elliptical form, and accordingly although as a practical matter we refer in this application to a distorting operation as representing the initial step in the prac- 145 150

tice of our present invention, we wish to call particular attention to the fact that it is quite possible to avoid this initial distorting step by the original production of non-circular tubing by the extrusion of lead from a press provided with elliptical or other non-circular dies. The significant part of our invention is the filling of a non-circular tube with a molten detonating agent and permitting this detonating agent to solidify in the tube while the tube is still of non-circular cross-section, and thereafter giving this tube a circular form with increase in cross-sectional area without significant change in perimeter or circumference, and the precise means by which the tubing is initially obtained in non-circular cross-section uniformly throughout its length is not an essential feature of our invention.

It will be evident that many modifications may be made within the limits of the disclosure as herein made, and accordingly no limitation of our invention should be made except as indicated in the appended claims.

We claim:

1. In the manufacture of detonating fuse the process which comprises filling a metal tube of non-circular cross-section throughout its effective length with a molten detonating agent, permitting the detonating agent to solidify while the tube remains non-circular in cross-section, distorting the tube to circular cross-section and decreasing the diameter and increasing the length of the filled tube to form cordeau therefrom.

35

110

40

115

45

120

50

125

55

130

60

135

65

140

70

145

75

150

2. In the manufacture of detonating fuse the process which comprises filling a metal tube of elliptical cross-section throughout its effective length with a molten detonating agent, cooling to solidify the detonating agent and thereafter applying pressure to the elliptical tube in the direction of its major axis to distort the tube to circular cross-section and thereafter decreasing the diameter and increasing the length of the filled tube to form cordeau therefrom.

3. In the manufacture of detonating fuse the process which comprises distorting a metal tube of circular cross-section to form tubing which is of non-circular cross-section uniformly over its effective length, filling the tube with a molten detonating agent, and permitting this molten detonating agent to solidify while the tube is of non-circular cross-section and thereafter restoring the filled tube to circular form and decreasing its diameter and increasing its length to form cordeau therefrom.

4. In the manufacture of detonating fuse the process which comprises charging a molten detonating agent into a metal tube the cross-sectional area of which is uniformly less than the cross-sectional area of a circle having a circumference equal to the perimeter of the tube, permitting the molten detonating agent to solidify, distorting the tube to circular cross-section and thereafter decreasing the diameter and increasing the length of the filled tube to form cordeau therefrom.

WALTER O. SNELLING.  
CLARENCE B. KOCH.